

2,791,526

## METHOD OF PRODUCING CASTINGS HAVING HIGH MECHANICAL PROPERTIES

Lucien Jules Péras, Billancourt, France, assignor to Régie Nationale des Usines Renault, Billancourt, France

No Drawing. Application July 7, 1954,  
Serial No. 441,923

Claims priority, application France August 27, 1953

10 Claims. (Cl. 148—21.7)

This invention relates to a method of producing castings having high mechanical properties.

It is known that in malleable iron castings, that is to say white iron castings treated thermally for the purpose of graphitisation, the graphite is obtained in nodular form, i. e., in the form of nodes or piles of very irregular form, and that owing to this fact the mechanical properties are appreciably lower than those of iron castings in which the graphite is spheroidal, this being obtained in direct fashion upon casting in the case of compositions which are either hypereutectic, comprising cerium, or which contain magnesium, usually in association with nickel.

It is known that sulphur interferes with the graphitisation of malleable iron castings, and that its effect must be neutralised by an excess of manganese, in which connection the ratio of Mn/S must be greater than 3.

Since an excess of manganese may interfere with the graphitisation, the manganese must be limited, and in consequence the position is similar with regard to sulphur, which usually remains at less than 0.15%.

It is furthermore known that sulfur lowers the mechanical properties of steel, so that with the exception of ordinary screw cutting steels containing manganese sulphide the lowest percentages of sulphur are usually sought, generally below 0.05%.

It is, therefore, paradoxical to endeavour to improve the properties of iron castings by a substantial increase in the sulphur with a corresponding reduction in manganese. It is accordingly a matter of surprise thus to arrive at mechanical properties which have not been obtained heretofore in graphitised white iron castings or, more generally, in iron castings free from alloyed substances. These means and the new and surprising results obtained represent the essential features of the present invention.

It has been made known heretofore that when the proportion of S/Mn in a white iron casting is increased the graphitisation upon annealing tends to change the graphite of nodular form in irregular heaps into a spheroidal form, in which the spherules are more and more symmetrical and regular. This scientific fact, however, has not heretofore acquired industrial significance, because the casting also comprised lamellar graphite, formed upon solidification, or irregular nodular graphite developed during annealing or, if only spheroidal graphite was involved, it was impossible to obtain complete transformation of the cementite caused by solidification, irrespective of the duration of the annealing process.

In each case the mechanical properties remained poor.

It is known that in malleable white iron castings a martensitic hardening facilitates fine graphitisation during the subsequent annealing process. It has shown previously, as a result of investigations, that this treatment reaches its full effectiveness when it is followed by a graphite crystal nucleus forming treatment at around 450° and of sufficient duration (10-50 hours) before

graphitisation is effected by annealing at high temperature.

In the sulphur castings forming the subject matter of the present invention the white iron obtained upon the pouring operation must also be subjected to a hardening process before annealing is performed for the purpose of graphitisation. However, in contradistinction to the preceding case, the crystal nuclear forming treatment should not be carried out, as it is not the object to multiply to a maximum the graphite nuclei capable of giving rise to fine nodules, but more probably to bring about nuclear formation of the graphite in the fine inclusions of iron sulphide.

According to the invention it is proposed to employ an iron casting rich in a finely distributed iron sulphide (FeS) content; to effect a martensitic hardening, the martensite formed giving rise by heating to unstable percarbides which are capable of subsequent conversion into cementite and graphite according to a reaction of the

20 type:



then to form the graphite nuclei by epistaxis on the hexagonal pyrites, and finally to permit free development of the nuclei to provide graphite spherules.

It may be remarked that if the formation of nuclei is concerned, the sole condition of similarity of the crystalline system suffices, a relation between the lattice dimensions not being necessary.

30 The invention, which permits in the case of cast iron, which is totally white upon the pouring operation, of a graphitisation upon annealing without the formation of cementite produced by solidification, resulting in a totally spherulitic graphite, is characterised by the following features:

(1) The composition comprises a proportion of S/Mn which is greater than 1—and more particularly less than 0.15 manganese and more than 0.2 sulphur, and preferably it is comprised within the following limits:

40  $\text{C}=2.10$  to  $2.70$   $\text{Si}=0.85$  to  $1.10$   $\text{Mn}=0.002$  to  $0.15$   
 $\text{S}=0.20$  to  $0.30$   $\text{P}=0.10$

Generally speaking, there are not special components.

(2) Solidification in the mould should take place as rapidly as possible, and preferably more rapidly than is strictly necessary to obtain the white structure. This leads to a fine distribution of the iron sulphide, on which there depends the fineness of distribution of the graphite spherules obtained during the course of the subsequent annealing process. Casting in a chill mould is preferable to casting in sand.

55 (3) The thermal treatment comprises essentially a martensite hardening or, if desired, an inferior hardening before carrying out the graphitisation by annealing.

This hardening is performed with advantage in conditions of rapid cooling, preferably for example in oil, or if desired in a bath of salts, which may be a fusible mixture of alkaline nitrate and alkaline nitrite and leads to a martensitic structure.

60 To avoid the danger of shrinkage upon hardening there has been recognised according to the invention the prime importance of effecting a preliminary annealing, a simple austenisation beyond termination of the transformation upon the heating  $A_1$  followed by cooling at a medium speed, such as cooling in still air.

According to the invention it has also been recognized that if the cooling for the purpose of solidification is moderate (casting in sand), it may be necessary to carry out two consecutive austenisation treatments with martensitic hardening.

(4) The thermal treatment furthermore comprises, following the martensitic hardening, a graphitisation an-

nealing beyond the point A<sub>1</sub>, i. e., at a temperature sufficiently high so that the casting will be constituted only by cementite and austenite, such temperature being maintained for a sufficient length of time to permit of total disappearance of the cementite not dissolved in the austenite at the annealing temperature. The duration of this annealing process is less than that in the case of usual white iron malleable castings annealed at the same temperature.

The consecutive cooling is carried out in accordance with the mechanical properties sought to be achieved. There may be obtained a total eutectoidal graphitisation in respect of a ferrite and graphite structure, as in malleable castings of the usual kind—very soft—or preferably the graphitisation may be stopped at such a point that the matrix has a substantially eutectoidal (lamellar perlite) composition, which leads to increased toughness.

Finally, it is possible as a subsequent step to carry out austenisation, quenching and tempering in order to obtain a greater toughness.

An example of reduction to practice of the method according to the invention is given in the following:

Pieces of metal having a weight of 700 grams and a mean thickness of 20 mm. are cast in moulds which are partially metal and partially composed of sand.

The castings have the following composition:

Carbon=2.5 Silicon=1 Manganese=0.12  
Sulphur=0.28 Phosphorus=0.10

Following stripping and complete cooling of the castings the latter are heated to 820° over a period of 30 minutes and are cooled in still air. There is thereupon carried out a second heating to 825° over a period of 30 minutes, and the pieces of metal are hardened in oil. The pieces are then reheated to 940° for a period of eight hours, after which they are removed from the furnace and cooled in still air.

A structure is obtained comprising fine graphite spherules on a lamellar perlite base.

Mechanical tests carried out on test pieces taken from these metal parts have produced the following results:

Tensile strength: 55 to 75 kg./mm.<sup>2</sup>

Breaking strength: 55 to 100 kg./mm.<sup>2</sup>

Elongation limit: 5 to 6%

Properties of this nature have not been obtained collectively heretofore in conjunction with castings devoid of all alloyed substances.

The limit of resistance to rotative bending has been measured in conjunction with Moore test pieces.

The resistance limit has been found to be 38 to 40 kg./mm.<sup>2</sup>, which is greater than that of the usual spheroidal castings.

The method referred to has the following advantages:

It is applicable to readily produced castings which make use of ores containing sulphur, and are of low commercial value, and it does not resort to any special substance alloyed therewith.

It provides, upon annealing, a very even distribution of graphite in the form of spherules, this structure being associated itself with very high mechanical properties, the breaking strength being between 95 and 105 kg./mm.<sup>2</sup> with an elongation of between 5 and 6.5% if the matrix is lamellar perlitic.

Its industrial application is economical and it can be readily utilised, leading to uniform nature of the results obtained.

What I claim is:

1. A process of thermally treating white castings to produce malleable iron with annealed spheroidal graphite therefrom, said castings containing 0.2 to 0.3% sulfur and 0.002 to 0.15 manganese with the ratio S/Mn being greater than 1, said process comprising the steps of heating said castings and directly quenching to impart a martensitic structure to the metal, and graphitization annealing at a temperature higher than that employed in the

heating step, said temperature being maintained until total disappearance of the cementite not dissolved in the austenite at the annealing temperature.

2. A process as defined in claim 1, wherein said castings also contain 2.1 to 2.7% carbon, 0.85 to 1.1% silicon and 0.1% phosphorus.

3. A process of thermally treating white castings to produce malleable iron with annealed spheroidal graphite therefrom, said castings containing 0.2 to 0.3% sulfur and 0.002 to 0.15 manganese with the ratio S/Mn being greater than 1, said process comprising the steps of heating said castings and directly quenching to impart a martensitic structure to the metal, and graphitization annealing at a temperature of 900 to 950° C. which is higher than that in the heating step, said annealing temperature being maintained for a period of 5 to 12 hours to effect total disappearance of the cementite not dissolved in the austenite at the annealing temperature.

4. A process of thermally treating white castings to produce malleable iron with annealed spheroidal graphite therefrom, said castings containing 0.2 to 0.3% sulfur and 0.002 to 0.15 manganese with the ratio S/Mn being greater than 1, said process comprising the steps of heating said castings to a temperature of about 820° C. for about thirty minutes, cooling in air, heating again to a temperature of about 825° C. for about thirty minutes, hardening in oil, reheating to about 940° C. for about eight hours, and cooling in air.

5. A process as defined in claim 1, wherein said castings are formed in semi-metallic molds.

6. A process of thermally treating white castings to produce malleable iron with annealed spheroidal graphite therefrom, said castings containing 0.2 to 0.3% sulfur and 0.002 to 0.15 manganese with the ratio S/Mn being greater than 1, said process comprising the steps of effecting a preliminary annealing of the castings and cooling in air, heating the thus annealed castings and directly quenching to impart a martensitic structure to the metal, and graphitization annealing at a temperature higher than that employed in the heating step, said temperature being maintained until total disappearance of the cementite not dissolved in the austenite at the annealing temperature.

7. A process of thermally treating white castings to produce malleable iron with annealed spheroidal graphite therefrom, said castings containing 0.2 to 0.3% sulfur and 0.002 to 0.15 manganese with the ratio S/Mn being greater than 1, said process comprising the steps of heating said castings and directly quenching to impart a martensitic structure to the metal, repeating said heating and said quenching, and graphitization annealing at a temperature higher than that employed in the heating step, said temperature being maintained until total disappearance of the cementite not dissolved in the austenite at the annealing temperature.

8. A process of thermally treating white castings to produce malleable iron with annealed spheroidal graphite therefrom, said castings containing 0.2 to 0.3% sulfur and 0.002 to 0.15 manganese with the ratio S/Mn being greater than 1, said process comprising the steps of heating said castings and directly quenching to impart a martensitic structure to the metal, graphitization annealing at a temperature higher than that employed in the heating step, said temperature being maintained until total disappearance of the cementite not dissolved in the austenite at the annealing temperature, and cooling said castings in air.

9. A process of thermally treating white castings to produce malleable iron with annealed spheroidal graphite therefrom, said castings containing 0.2 to 0.3% sulfur and 0.002 to 0.15 manganese with the ratio S/Mn being greater than 1, said process comprising the steps of heating said castings and directly quenching to impart a martensitic structure to the metal, graphitization annealing at a temperature higher than that employed in the

heating step, said temperature being maintained until total disappearance of the cementite not dissolved in the austenite at the annealing temperature, and quenching said castings.

10. A process of thermally treating white castings to 5 produce malleable iron with annealed spheroidal graphite therefrom, said castings containing 0.2 to 0.3% sulfur and 0.002 to 0.15 manganese with the ratio S/Mn being greater than 1, said process comprising the steps of heating said castings and directly quenching to impart 10 a martensitic structure to the metal, graphitization annealing at a temperature higher than that employed in the

heating step, said temperature being maintained until total disappearance of the cementite not dissolved in the austenite at the annealing temperature, repeating the first heating step, and directly quenching.

References Cited in the file of this patent

UNITED STATES PATENTS

|           |               |               |
|-----------|---------------|---------------|
| 1,542,440 | Drysdale      | June 16, 1925 |
| 1,932,664 | Hayes et al.  | Oct. 31, 1933 |
| 2,008,452 | Jewett et al. | July 16, 1935 |